

# United States Patent [19]

Bridger et al.

[11] 3,849,320

[45] Nov. 19, 1974

[54] **ORGANIC COMPOSITIONS CONTAINING  
ALKALI METAL ARYLCARBAMATES**

[75] Inventors: **Robert F. Bridger**, Hopewell;  
**El-Ahmadi I. Heiba**; **Stamoulis**  
**Stournas**, both of Princeton, all of  
N.J.

[73] Assignee: **Mobil Oil Corporation**, New York,  
N.Y.

[22] Filed: **Nov. 30, 1972**

[21] Appl. No.: **310,752**

[52] U.S. Cl. .... **252/33.6**, **252/42.7**

[51] Int. Cl. .... **C10m 1/54**

[58] Field of Search..... **252/42.7**, **33.6**, **397**

## [56] References Cited

### UNITED STATES PATENTS

2,629,694 2/1953 Woods et al..... **252/33.6**

|           |         |                   |                   |
|-----------|---------|-------------------|-------------------|
| 2,652,362 | 9/1953  | Woods et al.....  | <b>252/33.6</b>   |
| 3,056,820 | 10/1962 | Martinek .....    | <b>252/33.6 X</b> |
| 3,151,076 | 9/1964  | Epton et al. .... | <b>252/33.6</b>   |

*Primary Examiner*—H. Sneed  
*Attorney, Agent, or Firm*—Andrew L. Gaboriault;  
Raymond W. Barclay; Benjamin I. Kaufman

## [57] ABSTRACT

Organic compositions, particularly lubricating compositions in the form of lubricating oils and greases, are provided, containing, as antioxidants, alkali metal arylcarbamates.

**10 Claims, No Drawings**

## ORGANIC COMPOSITIONS CONTAINING ALKALI METAL ARYLCARBAMATES

### BACKGROUND OF THE INVENTION

#### 1. Field of the Invention

This invention relates to organic compositions having improved antioxidant properties. In one of its aspects, the invention relates, more particularly, to lubricant compositions in the form of lubricating oils and greases containing novel and improved antioxidant additives.

#### 2. Description of the Prior Art

Various antioxidant agents for use in organic compositions, particularly lubricants in the form of lubricating oils and greases have heretofore been suggested. In many instances, it has been found, however, that such antioxidants, e.g., amines or phenolic compounds, do not impart desirable alkaline properties to the lubricants. In other instances, such antioxidants do not exhibit a sufficiently effective degree of inhibiting oxidation. In general, therefore, these antioxidant additives have not proved to be sufficiently attractive to warrant any extensive industrial application.

### SUMMARY OF THE INVENTION

In accordance with the present invention, new and improved lubricant compositions in the form of lubricating oils and greases are provided, containing, as antioxidant agents, certain alkali metal arylcarbamates. More specifically, these carbamates comprise alkali metal arylcarbamates, diarylcarbamates and alkarylcarbamates having the structure:



in which  $R^1$  and  $R^2$  are phenyl, naphthyl, alkyl, aryl or hydrogen; at least one of  $R^1$  and  $R^2$  is aryl; and  $M$  is selected from the group consisting of Li, Na, K, Rb, Cs or tetraalkyl ammonium.

When the above-described carbamates are incorporated in organic media such as lubricant compositions, in the form of lubricating oils and greases, it is found that they impart a relatively high degree of improvement in alkalinity and are highly effective in inhibiting oxidation of the media into which they are incorporated. In general, the carbamates are employed in minor amounts. In most instances, the carbamates are effectively employed in amounts from about 0.001 to about 5%, and, preferably, from about 0.1 to about 2%, by weight, of the total weight of the lubricant composition.

The carbamate antioxidant may be effective incorporated in any oil of lubricating viscosity or in a grease composition in which the oil of lubricating viscosity is the vehicle in combination with a suitable thickening agent.

The lubricating oils which are improved with the antioxidants of the present invention may include mineral oils and synthetic oils of lubricating viscosities. Of particular significance is the improvement of petroleum distillate lubricating oils having boiling points as high as 650°F. or above and also mixtures of such oils. It should be noted, in this respect, that the term "distillate oils" is not intended to be restricted to straight-run distillate fractions. These distillate oils can be straight-run distillate oils, catalytically or thermally cracked (including hydro-cracked) distillate oils, or mixtures of straight-run distillate oils, naphthas and the like, with cracked distillate stocks and may be of varying viscosities and

pour points. Moreover, such oils can be treated in accordance with well-known commercial methods, such as acid or caustic treatment, hydrogenation, solvent-refining, clay treatment and the like.

As previously indicated, the aforementioned antioxidants may also be incorporated in grease compositions. Such greases, may comprise a combination of a wide variety of lubricating vehicles and thickening or gelling agents. Thus, greases in which the aforementioned carbamates are particularly effective may comprise any of the conventional hydrocarbon oils of lubricating viscosity, as the oil vehicle, and may include mineral oils or mineral oils in combination with synthetic lubricating oils, aliphatic phosphates, esters and di-esters, silicates, siloxanes and oxalkyl ethers and esters. Mineral lubricating oils, preferably employed as the lubricating vehicle, may be of any suitable lubricating viscosity range from about 45 S.U.S. at 100°F. to about 6,000 S.U.S. at 100°F., and, preferably, from about 50 to about 250 S.U.S. at 210°F. These oils may have viscosity indexes varying from below 0 to about 100 or higher. Viscosity indexes from 70 to about 95 are preferred. The average molecular weights of these oils may range from about 250 to about 800. The lubricating oil is employed in the grease composition in an amount sufficient to constitute the balance of the total grease composition, after accounting for the desired quantity of the thickening agent, and other additive components to be included in the grease formulation.

As hereinbefore indicated, the oil vehicles employed in the novel grease formulations, in which the aforementioned antioxidant carbamates are incorporated, may also comprise mineral oils or combinations of mineral oils with synthetic oils of lubricating viscosity.

When high temperature stability is not a requirement of the finished grease, mineral oils having a viscosity of at least 40 S.U.S. at 100°F., and particularly those falling within the range from about 60 S.U.S. to about 6,000 S.U.S. at 100°F. may be employed. In instances, where synthetic vehicles are employed in addition to mineral oils, as the lubricating vehicle, various compounds of this type may be successfully utilized. Typical synthetic vehicles include: polypropylene, polypropylene glycol, trimethylol propane esters, neopentyl and pentaerythritol esters, di-(2-ethyl hexyl) sebacate, di-(2-ethyl hexyl) adipate, di-butyl phthalate, fluorocarbons, silicate esters, silanes, esters of phosphorus-containing acids, liquid ureas, ferrocene derivatives, hydrogenated mineral oils, chain-type polyphenyls, siloxanes and silicones (polysiloxanes), alkyl-substituted diphenyl ethers typified by a butyl-substituted bis (p-phenoxy phenyl) ether, phenoxy phenyl ethers, etc.

The lubricating vehicles of the aforementioned improved greases containing the above-described antioxidant carbamates, are combined with a grease-forming quantity of a thickening agent. These thickening or gelling agents may include any of the conventional metal salts or soaps; which are dispersed in the lubricating vehicle in grease-forming quantities, in such degree as to impart to the resulting grease composition, the desired consistency. Other thickening agents that may be employed in the grease formation may comprise the non-soap thickeners, such as surface-modified clays and silicas, aryl ureas, calcium complexes and similar materials. In general, grease thickeners may be employed which do not melt and dissolve when used at the required temperature within a particular environment;

however, in all other respects, any materials which are normally employed for thickening or gelling hydrocarbon fluids for forming greases, can be used in preparing the aforementioned improved greases in accordance with the present invention.

The alkali metal arylcarbamates of the present invention, as more fully hereinafter described, may be prepared, in general, by reacting an arylamine, diarylamine or alkarylamine having the structure  $R^1R^2NH$  with a derivative of an alkali metal having the structure  $MX$  at a temperature from about  $0^{\circ}C.$  to about  $150^{\circ}C.$ , and preferably from about  $25^{\circ}C.$  to about  $60^{\circ}C.$ , to produce a product having the structure  $R^1R^2NM$ ; and reacting the product thus produced with carbon dioxide at a temperature from about  $0^{\circ}C.$  to about  $60^{\circ}C.$ , and preferably from about  $20^{\circ}C.$  to about  $30^{\circ}C.$ , to produce a product having the structure  $R^1R^2NCO_2M$  in which  $R^1$  and  $R^2$  are phenyl, naphthyl, alkyl, aryl or hydrogen; at least one of  $R^1$  and  $R^2$  is aryl;  $M$  is selected from the group consisting of Li, Na, K, Rb, Cs or tetraalkyl ammonium; and  $X$  is selected from the group consisting of  $-H$ ,  $-NH_2$ ,  $-N(CH_3)_2$ ,  $-C_6H_5$ , phenyl,  $-OH$ ,  $-OCH_2$ ,  $OC(CH_3)_2$  and  $-OC(CH_3)_2CH_2CH_2$ .

## DESCRIPTION OF SPECIFIC EMBODIMENTS

The following examples will serve to illustrate the novel alkali metal arylcarbamates of the present invention, the method for their preparation and their utility in organic lubricating media.

### Example 1

**Example 1:** N-Phenyl-1-naphthylamine (29.2 grams, 0.133 mole) was added to an ice-cooled solution of butyl lithium (12 grams, 0.187 mole) in 100 ml of tetrahydrofuran over a period of 30 minutes while the solution was stirred under an argon atmosphere. The rate of addition was determined chiefly by the heat evolved during the reaction. Stirring was continued for 30 minutes and

the solution was allowed to warm to room temperature. Dry carbon dioxide was pressed through the solution for 1 hour, and solvent was removed by evaporation in a vacuum. The product so obtained (39.6 grams), melting point 290°-292°C., was shown not to contain N-phenyl-1-naphthyl-amine by thin layer chromatography, and had minor impurities of lithium pentanoate and solvent. The N-H absorption was absent from the infrared spectrum which exhibited a carbonyl absorption at 6.2 microns. The compound, thus produced, had the following structure:



### Example 2

The procedure described in Example 1 was repeated, except that 34.1 grams of N-[p-(2,4,4-trimethyl-2-pentyl)phenyl]-1-naphthylamine and 7.5 grams of butyl lithium was employed. The resulting compound had the following structure:



### Example 3

10 The procedure described in Example 1 was repeated, except that 29.2 grams of N-phenyl-2-naphthylamine and 12 grams of butyl lithium was employed. The resulting compound had the following structure:



#### Example 4

**Example 4**  
The procedure described in Example 1 was repeated, except that 7.5 grams of butyl lithium and 16.9 grams of diphenylamine was employed. The resulting com-  
25 pound had the structure:



### Example 5

The procedure described in Example 1 was repeated, except that 7.5 grams of butyl lithium and 39.3 grams of di[p-(2,4,4-trimethyl-2-pentyl)phenyl]amine was employed. The resulting compound had the following structure:



#### 45 Example 6

Example 6  
A solution of 16.9 grams diphenylamine (0.1 mole) in 100 ml tetrahydrofuran was added, dropwise and with stirring, to a suspension of 4.2 grams sodium hydride (57% in mineral oil, washed with pentane) in 400 ml tetrahydrofuran. After the evolution of hydrogen had ceased, dry  $\text{CO}_2$  was passed through the solution for 30 minutes. Evaporation of the tetrahydrofuran afforded 21.2 grams (90%) of the sodium N, N-diphenylcarbamate, as a greyish solid, m.p.  $> 250^\circ\text{C}$ .  
This compound had the following structure:



### 65 Example 7

The procedure described in Example 6 was repeated, employing the same quantity of sodium hydride and 39.3 grams of di[p-(2,4,4-trimethyl-2-pentyl)phenyl]amine. The resulting compound had the following structure:



## Example 8

The procedure described in Example 1 was repeated, except that 6.8 grams of butyl lithium and 26.1 grams of dodecylaniline was employed. The resulting compound had the following structure:



## Example 9

The procedure described in Example 1 was repeated, except that 17.3 grams of 2,2,4-trimethyldihydroquinoline and 7.5 grams of butyl lithium was employed. The resulting compound had the following structure:



## Example 10

A solution of di [p-(2,4,4-trimethyl-2-pentyl)-phenyl]amine (19.65g., 0.05 mol) and potassium-tert-butoxide (5.61g., 0.05 mol) in 100 ml tetrahydrofuran was refluxed under an argon atmosphere for 22 hours. The resulting potassium salt precipitated from tetrahydrofuran. The tetrahydrofuran was replaced by adding 1,4-dioxane (200 ml) as the tetrahydrofuran was removed by distillation. A vigorous stream of carbon dioxide was passed through the solution for 1 hour. Upon evaporation of the solvent a yield of 26.9g. of product was obtained. The resulting product had the following structure:



## Example 11

To a solution of 4g. of the potassium carbamate of Example 10 in 75 ml acetonitrile was added 2.0g. of tetraethylammonium tetrafluoroborate. The solution was stirred 0.5 hours and filtered. To the filtrate was added 35 ml diethyl ether and the solution was filtered again. Evaporation of the solvent yielded 3.15g. of product. The resulting product had the following structure:



Individual blends of the carbamates of Examples 1 through 11 were prepared in Kuwait oil. This oil was prepared from a Kuwait distillate by furfural refining and methylethyl ketone dewaxing. It had a viscosity at

100°F. of 107 S.U.S. and at 210°F. of 40.1 S.U.S. Oxygen was circulated through each test sample at 175°C. at the rate of 5 liters per hour. The size of each sample was 30 grams. In the following table are summarized 10 the results as the time ( $t_{1.0}$ ) required for 1 kg of oil to absorb 1 mole of oxygen. In this table, the longer the duration of oxygen uptake, the more desirable the anti-oxidant carbamate additive. Where the carbamate additive was incorporated in the oil, it was present in an 15 amount of 1%, by weight.

TABLE

|    | CARBAMATE ADDITIVE | $t_{1.0}$ hours |
|----|--------------------|-----------------|
| 20 | Untreated oil      | 20 ± 2          |
|    | Oil + carbamate of |                 |
|    | Ex. 1              | 83.1            |
|    | do. Ex. 2          | 62.8            |
|    | do. Ex. 3          | 80.7            |
|    | do. Ex. 4          | 87.0            |
|    | do. Ex. 5          | 65.4            |
|    | do. Ex. 6          | 119.2           |
|    | do. Ex. 7          | 55.1            |
|    | do. Ex. 8          | 28.5            |
|    | do. Ex. 9          | 56.2            |
|    | do. Ex. 10         | 62.8            |
|    | do. Ex. 11         | 73.3            |

30 From the above examples and comparative data, it will be apparent that the alkali metal arylcarbamates of the present invention are outstandingly effective as anti-oxidants in organic media such as lubricating oils, and greases in which these lubricating oils are employed as vehicles. It will also be noted that other additives may also be included in the above-described organic compositions which can provide a variety of additional desirable characteristics such as extreme pressure agents, detergents, pour point depressants, stability improvers and viscosity control agents.

35 40 While preferred embodiments of the novel process of the present invention have been described for the pur-

poses of illustration, it will be understood that various modifications and adaptations thereof, which will be obvious to those skilled in the art, may be made without departing from the spirit of the invention.

We claim:

55 1. A lubricant composition containing, as an antioxidant, a minor amount of a carbamate of the group consisting of alkali metal arylcarbamates, diarylcarbamates and alkarylcarbamates having the structure:



in which  $R^1$  and  $R^2$  are alkyl, aryl or hydrogen; at least one of  $R^1$  and  $R^2$  is aryl; and  $M$  is selected from the

group consisting of Li, Na, K, Rb, Cs or tetraalkyl ammonium.

2. The composition of claim 1 wherein said composition comprises an oil of lubricating viscosity.

3. The composition of claim 1 wherein said composition comprises a grease.

4. The composition of claim 1 containing from about 0.001 to about 5%, by weight, of said antioxidant.

5. The composition of claim 1 containing from about 0.1 to about 2%, by weight, of said antioxidant.

6. The composition of claim 1 wherein said antioxidant has the structure:

8. The composition of claim 1 wherein said antioxidant has the structure:



9. The composition of claim 1 wherein said antioxidant has the structure:



10. The composition of claim 1 wherein said antioxidant has the structure:



7. The composition of claim 1 wherein said antioxidant has the structure:



\* \* \* \* \*